

Dec. 19, 1939.

L. B. LINDEMUTH

2,183,576

CASTING STEEL INGOT

Filed May 26, 1936

*Fig. 1.*



*Fig. 2.*



*Fig. 3.*



INVENTOR.

LEWIS B. LINDEMUTH.

BY *Minar Rauber*

ATTORNEYS

## UNITED STATES PATENT OFFICE

2,183,576

## CASTING STEEL INGOT

Lewis B. Lindemuth, Port Washington, N. Y.

Application May 26, 1936, Serial No. 81,806

9 Claims. (Cl. 22—216)

In certain previous applications, Ser. Nos. 712,-  
729 and 712,730, filed February 24, 1934, I have  
described apparatus and processes of casting in-  
gots by which to eliminate or greatly reduce the  
usual piping and segregation which have necessi-  
tated the cropping of a considerable percentage  
at the upper end.

The present invention is directed to similar  
purposes. Embodiments of the invention are  
10 illustrated in the accompanying drawing.

Fig. 1 is a vertical section through the up-  
per part of an ingot mold; Fig. 2 is a similar  
view illustrating a modification and Fig. 3 is a  
plan of the retainer of Fig. 2.

15 The purpose of the invention is to retain the  
heat in the top part of the cast metal so as  
to keep it fluid. I propose for this purpose to  
apply on top of the hot metal 1 in the ingot  
mold 2 a layer of ground cork 3.

20 This may be ground to any size, from dust to  
say particles of one-half inch. In order to re-  
tard the normal burning rate of the cork it is  
preferably impregnated by admixture with a  
small amount of water glass or silicate of soda;  
25 which can vary, for example, from five to twenty  
per cent by weight of the cork. Insofar as we  
keep the surface of the molten metal deoxidized,  
it will solidify less rapidly than an oxidized sur-  
face. It is preferable, therefore, to incorporate  
30 into the cork-water glass mixture a small  
amount, say one per cent, of some deoxidizing  
agent such, for example, as ferro-silicon or pow-  
dered aluminum. As the cork burns the deox-  
idizer falls on to the surface of the liquid metal  
35 and prevents the formation of a film of oxide  
on it. The cork, of course, is a heat insulating  
material and itself assists in maintaining a re-  
ducing or non-oxidizing atmosphere on top of the  
ingot.

40 A great advantage in the use of cork arises  
from its lightness. The total carbon content of  
the weight of cork used is insufficient to alter the  
composition of the top of the ingot. This is true  
even though the ingots are refilled, as described  
45 in my application (712,729), and the metal for  
refilling poured through the cork or mixture on  
the top of the ingot.

Using the mixture of cork, silicate of soda, and  
50 ferro-silicon on an ingot twenty inches square,  
a quantity between one-half and one cubic foot  
is sufficient to maintain the top of an ordinary  
open-hearth steel ingot fluid for a period of  
thirty to sixty minutes. Such a quantity of the  
55 mixture represents a layer varying from about  
two to four and one-half inches in depth.

The invention has particular value in casting  
ingots of rimming steel. By maintaining the  
surface in an unoxidized condition and insulated  
against cooling losses, the steel will remain fluid  
and will rim for a longer period, therefore pro-  
ducing a thicker skin on the ingot. In such  
steel there is a continued circulation of gases.  
The cork layer by extending the period of fluidity  
also extends the period during which the circula-  
tion continues. The lightness of the cork 10  
tends to prevent its being drawn down into the  
metal by the circulatory movement thereof. And  
the quantity of carbon contained is so slight, as  
explained above, as not to affect the composi-  
tion of even the upper part of the ingot.

15 Other materials have been proposed and even  
used for similar purposes but they have burned  
away too quickly or have supplied too great a  
quantity of carbon or have presented other dis-  
advantages in casting ordinary steel and have  
been practically useless in casting rimming steel.

20 Where there is to be a second teeming of hot  
metal into the top of the ingot, I preferably use  
the scheme shown in Figs. 2 and 3. A retainer  
4 having a widened base 5 is placed on top of  
the primary teeming. It fits loosely in the mold  
25 and floats on the metal, its broadened base en-  
suring that it shall enter only to a slight depth  
into the metal. The layer of cork or mixture  
3 is applied to the surface of the metal within  
the retainer 4 and the secondary teeming is  
30 poured through said layer. This is the method  
of my above cited application (712,729) with  
the addition of the layer 3 to hold the heat.

35 Various other modifications may be made by  
those skilled in the art without departing from  
the invention as defined in the following claims.

I claim:

1. The method of casting steel ingots which  
includes pouring the molten steel into the ingot  
40 mold and applying to the top a layer of ground  
cork to retard the cooling of the top of the cast  
metal.

2. The method of casting steel ingots which  
includes pouring the molten steel into the ingot  
45 mold and applying to the top a layer of ground  
cork mixed with a combustion retardant to re-  
tard the cooling of the top of the cast metal.

3. The method of casting steel ingots which  
includes pouring the molten steel into the ingot  
50 mold and applying to the top a layer of ground  
cork mixed with a deoxidizing agent to retard  
the cooling of the top of the cast metal.

4. The method of casting steel ingots which  
includes pouring the molten steel into the ingot 55

mold and applying to the top a layer of ground cork to a depth of about two to five inches to retard the cooling of the top of the cast metal.

5. The method of casting ingots of rimming steel which includes pouring the molten steel into the ingot mold and applying ground cork to the top to retard the cooling of the top of the cast metal and extend the period of rimming.

6. The process of claim 1 followed by a second <sup>10</sup> pouring of molten steel through the layer of cork.

7. The process of claim 1 followed by the application of a floating retainer and a second pouring of molten steel through the layer of cork <sup>15</sup> within the retainer.

8. The method of casting steel ingots which

includes pouring the molten steel into the ingot mold and applying to the top a layer of ground cork impregnated with silicate of soda to the extent of about 5 to 20 per cent by weight of the cork to retard the cooling of the top of the cast <sup>5</sup> metal.

9. The method of casting steel ingots which includes pouring the molten steel into the ingot mold and applying to the top a layer of ground cork impregnated with silicate of soda to the <sup>10</sup> extent of about 5 to 20 per cent by weight of the cork with which is incorporated a small percentage of a deoxidizing agent to retard the cooling of the top of the cast metal.

<sup>15</sup>

LEWIS B. LINDEMUTH.